

## UNITED STATES PATENT OFFICE

2,079,780

## WASHABLE PAPER

Robert A. Voet, Oak Park, Ill., assignor to United  
Wall Paper Factories, Inc., Jersey City, N. J., a  
corporation of Delaware

No Drawing. Application July 27, 1934,  
Serial No. 737,207

2 Claims. (Cl. 91—67.9)

My invention has to do broadly with arts wherein a protein such as casein, albumin, glue, and the like are used. Such arts, for example, include the coating of paper and the like, formation of films, webs and binders for pigments, the application of wood-joining glues, etc. An important field in which protein, particularly casein, binders are used is in the manufacture of water-proof wall paper, wherein casein is usually used 10 as a binder for the pigment and also as a water-proof coating for the printed paper.

It has been customary for a long time in using such adhesives to harden or set them by means of formaldehyde, either in the form of a gas or 15 as a strong aqueous solution, which has been incorporated with, sprayed upon, or otherwise applied to the solubilized or solubilized and dried protein. However, the use of formaldehyde has always been highly objectionable from a manu- 20 facturing standpoint because of the irritating effect of the gas on the mucous membrane, eyes and epidermis of workmen. This condition has required considerable expense to the manufacturer for equipment designed to reduce the discomfort 25 of workmen as much as possible.

An object of my invention is to produce a hardening or setting agent for protein materials of the type referred to above which is as effective as formaldehyde and at the same time avoids the 30 irritating effects on the workmen above referred to. I have been successful in evolving such a setting or insolubilizing agent which completely eliminates these disadvantages of formaldehyde and is sufficiently inexpensive to be commercially 35 attractive.

I have found that a solubilized protein may be insolubilized, i. e., set or hardened, by means of a solution containing formic acid, combined with 40 an alkaline reacting metal or metalloid, such as

I am aware that aluminum acetate has previously been suggested as a hardening agent for solubilized proteins. However, this material leaves a distinct acetic acid (vinegar) odor on the hardened and dried material. It is, therefore, objectionable. In accordance with my invention, on the other hand, substantially no odor remains.

## PREPARATION OF HARDENING SOLUTION

## Example I

The following is a preferred example of a hardening or setting solution prepared in accordance with my invention:

To 20 parts of water at 75° C., add 5 parts of aluminum formate. When this has completely dissolved, dilute with 75 parts of cold water. Then, if it is necessary to change the acidity phase of the solution, this can be done by careful use of a suitable alkali such as sodium hydroxide, but a careful check should be made with a sensitive type of pH indicator. For best results, the pH value should not exceed 5.5.

## Example II

To 20 parts of water at 75° C. add 4 parts by weight of paper-makers' iron-free alum. Dilute with 71 parts cold water in which 5 parts of sodium formate has previously been dissolved. Check with a sensitive indicator, such as Brom-Cresol Green, to adjust the pH between 5.5 and 4.8.

## Other examples

According to the general methods above described, other chemicals may be substituted for the materials specified in the two preceding examples. Among such other chemicals which may be employed, are those set forth in the following table of examples, commercial grades of the specified chemicals being referred to in each instance:

| Example No. |                          | Parts by wt. |                       | Parts by wt. | Water parts by wt. | pH of final solution |
|-------------|--------------------------|--------------|-----------------------|--------------|--------------------|----------------------|
| 45          | 3 Potassium formate..... | 5            | Aluminum sulfate..... | 2            | 93                 | 4.8                  |
|             | 4 Potassium formate..... | 5            | 90% formic acid.....  | 1/2          | 94 1/2             | 4.8                  |
|             | 5 Magnesium formate..... | 5            | Aluminum sulfate..... | 2            | 93                 | 4.9                  |
|             | 6 Magnesium formate..... | 5            | 90% formic acid.....  | 1/2          | 94 1/2             | 4.9                  |
|             | 7 Calcium formate.....   | 5            | Aluminum sulfate..... | 2            | 93                 | 4.9                  |
|             | 8 Calcium formate.....   | 5            | 90% formic acid.....  | 1/2          | 94 1/2             | 4.9                  |
|             | 9 Barium formate.....    | 5            | Aluminum sulfate..... | 1/2          | 93 1/2             | 4.8                  |
|             | 10 Barium formate.....   | 5            | 90% formic acid.....  | 1/4          | 94 1/4             | 4.8                  |
| 50          | 11 Sodium formate.....   | 5            | Aluminum sulfate..... | 1/2          | 94 1/2             | 4.8                  |
|             | 12 Aluminum formate..... | 5            | Sodium carbonate..... | 1/4          | 93 1/4             | 4.9                  |
|             | 13 Ammonium formate..... | 5            | Aluminum sulfate..... | 1/2          | 93 1/2             | 4.9                  |
|             | 14 Ammonium formate..... | 5            | 90% formic acid.....  | 1/4          | 93 1/4             | 4.9                  |

55 aluminum, sodium, potassium, calcium, magnesium, barium, or ammonium, said solution being made slightly acid, i. e., acid down to a limit of approximately pH 4.8, and preferably between the approximate limits of 5.5 and 4.8. The acidity is preferably produced by the  $SO_4$  radical.

## APPLICATION OF HARDENING SOLUTION TO MANUFACTURE OF WATER-PROOF WALL PAPER

To form the solubilized protein binder, soak 20 parts of dry casein and 75 parts of water for half an hour. Then while agitating the mixture, 60

raise the temperature to 48° C. At this point, add 4 pounds borax in sufficient amount of water to dissolve it. When all lumps and undissolved particles disappear and the solution cools, it is 5 ready for use by incorporating it with the other materials, such as clay, color pigments, bronze powders and dry mica to form the coating material, and the color inks. It is usual to have the micas and bronzes pulped beforehand with some 10 type of a low starch content gum, e. g., gum tragacanth, which tends to act both as a dispersing agent and a colloidal suspender.

The paper web is formed with a filler containing 15 solubilized casein, and is partially or wholly dried in the usual way.

The coating material, e. g., clay, suspended in the protein binding agent above referred to, is spread evenly over one side of the web of paper and dried usually by passing it through a drying 20 rack in festoons where ducts supply hot air which drives off the moisture in the coating, leaving the clay and color pigments firmly bound to the web by the thus solubilized-and-dried protein binder.

25 Next, the color inks made up with said protein binder, are printed upon the coated surface of the web and dried in the same manner as the coating was. Then, by using brushes or a roller appliance, the hardening agent in aqueous solution, prepared in accordance with my invention, is applied to the coated and printed surface of the web and again the moisture is evaporated off of the thus treated surface.

30 The degree of water resistance obtained by 35 using this hardening agent is of first-class quality and, in addition, any possible effect upon the paper fibers or printed colors is more negligible than when formaldehyde or formaldehyde and alum in solution is used.

#### 40 ALTERNATIVE EMBODIMENT

Instead of applying the setting solution to the protein coating as described above, I may combine it with the protein in dry form and dissolve 45 as required. The following example is illustrative:

Seventy parts of 30-mesh casein, 10 parts borax, 5 parts hydrated lime, 5 parts aluminum formate, and 5 parts sodium fluoride are thoroughly 50 mixed and passed through a 30-mesh screen. The dry mixture thus produced may be shipped in dry form and placed in solution as needed. For the quantities given above, add 400

parts of water and heat to 50° C. and agitate until thoroughly dissolved. The material just described is useful as an adhesive and could be combined with pigments and the like to give a water-resistant coating when applied to a web. 5

In this composition the borax and lime serve as the alkaline agents, in accordance with my invention, while borax also acts as a preservative of the protein and lime, furthermore, gives the glue high strength. The sodium fluoride acts as 10 a retarder to prevent immediate precipitation of the protein by the aluminum formate.

Various other modifications of my invention may suggest themselves to those skilled in the art without departing from the spirit of my invention and, hence, I do not wish to be limited to the specific embodiments disclosed herein, except to the extent indicated by the appended claims, which are to be interpreted as broadly as the state of the art will permit. Methods will 20 be obvious to those skilled in the art, without giving additional detailed examples, for preparing other hardening solutions embodying my invention and including one or more of the metals or metalloids specified above, and adjusted to the 25 specified acidity.

I claim as my invention:

1. A method of preparing an article of the class described, comprising treating a paper web with a coating containing solubilized casein as a potentially water resistant binder, at least partially drying the paper web, printing upon said web with an ink also containing a potentially water 30 resistant casein binder, and treating said web to fix said binders and render the surface of the paper water resistant by means of a solution of a formic acid salt of a member of the group consisting of alkali and alkaline earth metals, ammonium and aluminum, said solution having been adjusted to a pH value between the approximate 35 limits of 4.8 and 5.5. 40

2. A method of preparing water-resistant paper comprising treating a paper web with a coating composition containing a solubilized casein binder, at least partially drying said web, and insolubilizing said binder with a solution of a formic acid salt of a member of the group consisting of alkali and alkaline earth metals, aluminum and ammonium, said solution having been adjusted to a pH value between the approximate 50 limits of 4.8 and 5.5. 45

ROBERT A. VOET.